

June 20, 1950

A. R. LINDSAY

2,512,348

METHOD OF MAKING DIELECTRIC STENCILS

Filed Sept. 23, 1948



INVENTOR.  
Allen R. Lindsay  
BY  
Chas. H. Trotter  
Atty.

## UNITED STATES PATENT OFFICE

2,512,348

## METHOD OF MAKING DIELECTRIC STENCILS

Allen R. Lindsay, Cleveland Heights, Ohio

Application September 23, 1948, Serial No. 50,758

5 Claims. (Cl. 101—128.2)

1

This invention relates to a method of making dielectric stencils such as the stencil disclosed in my co-pending application Serial No. 50,757, filed September 23, 1948.

These stencils are used in conjunction with electrical etching tools for marking metallic articles such as tools, machines and various parts thereof.

The stencil is formed from a composite sheet of material and has the desired character impressed into the bottom thereof. In use the stencil is secured to a suitable etching tool and brought into contact with the article to be marked. The impression defining the character is then filled with a suitable electrolyte which is generally contained in a reservoir in the tool. An electric current is then passed through the electrolyte and into the article, the stencil holder or tool acting as the cathode and the article constituting the anode. One form of such an etching tool is shown in my co-pending application Serial No. 631,401, filed November 28, 1945, which has matured into Patent No. 2,498,129 Feb. 21, 1950. The actual etching time is very short, just a few seconds, so that a large number of articles can be marked in a short time. As the stencil is repeatedly brought into engagement with articles to be marked, which very often have a rough surface, it is subjected to mechanical abrasion which eventually wears out the stencil so that it has to be replaced with a new stencil.

The principal object of this invention is to provide a method of making dielectric stencils, for use with electrical etching devices, which are so constructed that they will resist mechanical abrasion and will have a much longer life than previously known stencils of this character.

Another object of the invention is to provide a method of making stencils which can be repeatedly used many times and will produce a clear cut well defined mark on a metallic article.

Another object of the invention is to provide a simple, economical and efficient method of making stencils having the aforesaid characteristics.

Other and more limited objects of the invention will be apparent from the following specification and the accompanying drawing forming a part thereof wherein:

Fig. 1 is a side elevation of a dielectric stencil made according to my improved method;

Fig. 2 is a bottom plan view thereof;

Fig. 3 is a greatly enlarged fragmentary section taken on the line 3—3 of Fig. 2;

2

Fig. 4 is an enlarged fragmentary section through the paper used in making the stencil;

Fig. 5 is a detail sectional view showing one way of applying a thin film of wax to one side of the paper;

Fig. 6 is an enlarged fragmentary section showing a thin film of wax applied to one side of the paper;

Fig. 7 is a view similar to Fig. 6 showing a thin film of buna rubber applied to the wax film;

Fig. 8 is an enlarged sectional view showing the manner of impressing a character into the composite sheet of paper, wax and buna rubber; and

Fig. 9 is a detail view showing one way of curving and vulcanizing the film of buna rubber around the character.

Referring now to the drawings by reference characters, the numeral 1 indicates generally a stencil made according to my improved method.

20 The stencil 1 comprises a flat bottom wall 2 and an annular wall 3 integral therewith. The upper end of the annular wall 3 is flared outwardly as indicated at 4. The mark or character 5 to be etched is impressed into the bottom wall 2 of the 25 stencil. A raised border 6 surrounds the mark or character 5. Although I have illustrated the stencil as generally circular in shape, it will be obvious to anyone skilled in this art that it can be square, rectangular or any other desired shape, depending on the size and shape of the mark desired and on the type of etching tool with which the stencil is used. Also the stencil need not be cup-shaped as shown. In some instances it may be desirable to make the stencil in the form of a 30 flat sheet.

The stencil is made from a composite sheet of material 7 which is first molded into shape, after which the desired mark or character 5 is impressed into the bottom wall 2 thereof by a suitable die.

35 The material 7 comprises a treated paper sheet 8, a thin film of wax 9 and a thin film 10 of high temperature paraffin and buna rubber, all firmly bonded together into a composite sheet. The paper 8 is preferably uncoated long fibre paper having extremely open tissues so that it is very 40 pervious and will allow electrolyte to readily pass through.

In making the stencil I first treat the paper 8 45 with chlorinated oil which seals the hygroscopic fibres and bonds them together. Then I apply the thin film of wax 9 to one side of the paper. In applying the film 9 I first dissolve paraffin and an animal wax in a suitable solvent, such as ether, 50 which has been heated to approximately 160°.

Then I pass the paper 8 over a chilled roller 11 which dips into the wax solution 12 in the container 13. As the paper 8 passes over the chilled roller 11 and through the solution 12 the roller 11 cools the paper and causes the thin film 9 to freeze onto the paper and firmly bond therewith. Next I spray an emulsion of high temperature paraffin and buna rubber onto the film 9 with a hot blast air gun 14. As the emulsion comes into contact with the wax film it solidifies into the thin film of paraffin and buna 10.

The stencil 1 is then molded from the composite sheet 7, with the films 9 and 10 on the outside of the stencil. After the stencil has been molded to form, I impress the desired mark or character 5 into the bottom thereof with a suitable die 15 as indicated in Fig. 8. As the die 15 is forced into the material it ruptures and displaces the films 9 and 10 and forms the raised border 6 around the character. The die also compresses the paper 8 thereunder which forces all wax and oil out of the compressed portion, leaving bare fibre through which electrolyte can readily pass. After the character has been impressed I fill the impression with electrolyte and then pass an electric current through the electrolyte. This generates enough heat to cure and vulcanize the film of buna rubber around the mark which gives the buna film high mechanical strength and provides a tough tenacious film which resists mechanical abrasion. The simplest way to cure and vulcanize the buna film is to secure the stencil to an etching tool 16 and use it once or twice to mark an article 17, as shown in Fig. 9.

From the foregoing it will be apparent to any one skilled in this art that I have provided a very simple, economical and efficient method of making dielectric stencils for use in etching marks upon metallic articles. In practice it has been found that a stencil made according to my method can be used 1900 times before it is worn beyond a desirable working point. Other known stencils when used in the same manner averaged only 30 times.

It is to be understood that I am not limited to the specific method shown and described herein as various modifications can be made thereto within the scope of the appended claims.

Having thus described my invention, I claim:

1. The method of making a dielectric stencil comprising, applying a thin film of animal wax to one side of a sheet of uncoated long fibre open tissue paper, applying a thin film of high temperature paraffin and buna rubber to the wax film, molding a stencil from the composite sheet thus formed, impressing a character into said sheet by forcing a die thereinto in such a manner as to rupture and displace the wax film and the buna rubber film, filling said character with electrolyte, and then passing an electric current through said electrolyte thereby generating sufficient heat to vulcanize the buna rubber film surrounding said character.

2. The method of making a dielectric stencil comprising treating a sheet of uncoated long fibre open tissue paper with chlorinated oil to seal the hygroscopic fibres and bind them together, coating one side of said sheet with a film containing

synthetic rubber, molding a stencil from said coated sheet, impressing a character into said sheet in such a manner as to rupture and displace said film, filling said character with electrolyte, and then passing an electric current through said electrolyte thereby generating sufficient heat to vulcanize the film surrounding said character.

3. The method of making a dielectric stencil comprising, treating a sheet of uncoated long fibre open tissue paper with chlorinated oil to seal the hygroscopic fibres and bind them together, coating one side of said sheet with a film containing animal wax, applying a second film which contains synthetic rubber to said first mentioned film, molding a stencil from the composite sheet thus formed, impressing a character into said sheet by forcing a die thereinto in such a manner as to rupture and displace the wax film and the buna rubber film, filling said character with electrolyte, and then passing an electric current through said electrolyte thereby generating sufficient heat to vulcanize the buna rubber film surrounding said character.

25 4. The method of making a dielectric stencil comprising, coating one side of a sheet of uncoated long fibre open tissue paper with a film containing buna rubber, molding a stencil from said coated sheet, impressing a character into said sheet in such a manner as to rupture and displace said film, filling said character with electrolyte, and then passing an electric current through said electrolyte thereby generating sufficient heat to vulcanize the film surrounding said character.

30 5. The method of making a dielectric stencil comprising, treating a sheet of uncoated long fibre open tissue paper with chlorinated oil to seal the hygroscopic fibres and bind them together, freezing a solution of paraffin and animal wax into a film on one side of said paper sheet, spraying an emulsion containing high temperature paraffin and buna rubber onto said film, said emulsion solidifying into a second film which is firmly bonded to said first mentioned film, molding a stencil from the composite sheet thus formed, impressing a character into said sheet by forcing a die thereinto in such a manner as to rupture and displace said films, filling said character with electrolyte, and then passing an electric current through said electrolyte thereby generating sufficient heat to vulcanize a portion of said second film which surrounds said character.

55 ALLEN R. LINDSAY.

#### REFERENCES CITED

The following references are of record in the file of this patent:

#### UNITED STATES PATENTS

| Number    | Name     | Date          |
|-----------|----------|---------------|
| 1,293,983 | Thomas   | Feb. 11, 1919 |
| 1,371,157 | Gesetner | Mar. 8, 1921  |
| 1,633,072 | Davis    | June 21, 1927 |
| 2,140,506 | Canning  | Dec. 20, 1938 |
| 2,405,508 | Lindsay  | Aug. 6, 1946  |